

# UNITED STATES PATENT OFFICE.

WALTER THEODORE FELS, OF MOUNT VERNON, NEW YORK, ASSIGNOR OF ONE-HALF  
TO JACOB FERBER, OF MOUNT VERNON, NEW YORK.

## PLASTIC COMPOSITION.

1,419,665.

Specification of Letters Patent. Patented June 13, 1922.

No Drawing.

Application filed January 14, 1921. Serial No. 437,316.

To all whom it may concern:

Be it known that I, WALTER T. FELS, a citizen of the United States, residing at Mount Vernon, in the county of Westchester 5 and State of New York, have invented certain new and useful Improvements in Plastic Compositions, of which the following is a specification.

The present invention relates to plastic 10 compositions, such as used for building purposes for the interior or exterior finish of walls, partitions, and the like.

The invention has for its object the provision of a novel and improved plastic composition which can be used to advantage for the production of composition boards, slabs or sheets which will have the qualities of strength, durability, sound-insulation, and low cost of manufacture, as well as being 20 readily worked, that is, the boards or slabs can be readily cut with a saw or other suitable implements and can be readily nailed or otherwise fastened to the studs or the like.

In carrying out the invention, the composition comprises the ingredients, as follows:—

|                  |     |
|------------------|-----|
| Locomotive ashes | 60% |
| Plaster Paris    | 30% |
| Lime             | 9%  |
| Glue             | 1%  |

Such materials are thoroughly mixed and are moistened with water sufficiently to render the mass homogeneous. Such proportions are approximate, inasmuch as they can be varied somewhat, but by adhering to such proportions substantially as given, the resultant product is a thoroughly efficient and useful one.

The glue used is prepared by cooking a suitable quantity of any preferred glue about 40 24 hours in plenty of water and lime amounting to about 10%, by volume, of the glue. Such solution, when boiled for about one

day, will form an effective glue to be used 45 in mixing the composition and making the same solid when it sets. The ingredients are preferably measured by volume, although the proportions will be substantially the same if measured by weight.

After the ingredients are mixed and worked thoroughly, the material can be worked or molded into boards, sheets or slabs of suitable size and thickness and when the material has set or become dry, it can 50 be cut into pieces and nailed or otherwise fastened to the studding or the like, to take the place of lathing and plaster or mortar, with a considerable saving in cost. The locomotive ashes can be obtained at small 55 expense, being a waste product and constituting a greater portion of the composition. Inasmuch as the boards or slabs can be readily cut and nailed or otherwise fastened to the studding, this provides for a considerable 60 saving, as over the old method of applying lathing and plaster. Furthermore, the boards or slabs are strong and durable, and also serve as sound-insulation, inasmuch 65 as the use of the ashes will deaden the transmission of sound through the boards or slabs.

The locomotive ashes are specially desirable and efficient, although there may be other ashes or cinders which would suffice 70 under certain conditions.

Having thus described the invention, what is claimed as new is:—

1. A plastic composition comprising in approximate proportion, 60% ashes, 30% 80 plaster Paris, 9% lime and 1% glue.

2. A plastic composition comprising in approximate proportion, 60% locomotive ashes, 30% plaster Paris, 9% lime and 1% glue.

In testimony whereof I hereunto affix my signature.

WALTER THEODORE FELS.